

2,957,778

## BRIGHTENING AND STABILIZING THE COLOR OF METAL SALTS OF NAPHTHENE- AND ETHYLHEXANIC ACIDS AND THEIR SOLUTIONS

Arnold Albers and Ernst Voss, Frankfurt am Main, Germany, assignors to Farbwerke Hoechst Aktiengesellschaft vormals Meister Lucius & Brüning, Frankfurt am Main, Germany, a corporation of Germany

No Drawing. Filed Feb. 17, 1958, Ser. No. 715,835

Claims priority, application Germany Feb. 22, 1957

6 Claims. (Cl. 106—310)

The present invention relates to a process for brightening and stabilizing the color of metal salts of the naphthene- and ethylhexanic acids and their solutions.

It is known that naphthenic acids and alpha-ethylhexanic acid, their metal salts and their solutions have a tendency to change color, or more especially, they readily turn dark upon heating. This applies especially to naphthenic acid with a low acid number and to the metal salts of this acid. The darkening is partially due to a certain content of sulfur in the naphthenic acids, and it has been proposed to eliminate such sulfur, for example by heating the acids in the presence of hydrogen peroxide or another peroxide, although alpha-ethylhexanic acid and naphthenic acids free from sulfur or having been freed from sulfur are also subject to similar darkening phenomena.

Moreover, it has already been described in the literature to admix metal salts of naphthenic acids with polyamines, aminophenols and other antioxidants, which most frequently contain nitrogen, so as to bring about a color-stabilization. These substances are, however, known to oxidize readily and to turn dark; moreover, they are very unstable, especially in the heat. Due to this instability, they are effective only for a relatively short time and they exhibit only an inferior stabilizing effect, especially at a raised temperature.

Attempts have also been made to obtain brighter colored metal salts of naphthenic acid by distilling off accompanying substances which have a great extinction coefficient, especially iron naphthenate. Such purification (distillation) is expensive and although it is true that it brightens the color of the starting material, it cannot prevent the dried substances from darkening, especially when they are subjected to a thermal treatment.

The darkening interferes with those metal salts which normally have a light color and serve as driers for making light colors, varnishes or lacquers. For example, darkened lead or calcium driers cannot be used as naphthenates or salts of ethylhexanic acid for making especially light colored lacquers. The same applies to other metal salts of the aforesaid acids, for example, zinc, cerium, lanthanum or zirconium salts, and for example, zirconyl salts or salts of similar metals.

Now, we have found that the darkening of metal salts, for example, the salts of the aforesaid metals and the darkening of solutions of these metal salts must be attributed to a catalyzed decomposition of the respective acids, a phenomenon which can be inhibited by admixing the metal salts with certain additions. In accordance with our invention, the metal salts to be stabilized or their solutions are admixed with tin salts soluble in these solutions. It is especially preferred to use the tin salts of naphthenic acid or alpha-ethylhexanic acid (octanic acid), but there may also be used the tin salts of other acids, for example, resin acids.

The use of a tin salt of the same acid which also appears in the metal salts to be stabilized involves the advantage that

(a) Apart from tin metal, no foreign substances appear in the drier, and that

(b) All other properties of the metal salts or their solutions, such as drying effect and clear solubility, are preserved.

In addition thereto, the aforesaid tin salts involve the advantage of being not-volatile, so that their effect cannot be lost prematurely by evaporation.

The tin salts of alpha-ethylhexanic acid are altogether somewhat more effective than the salts of naphthenic acid or resin acids, but the latter may also be used with good success. It is also possible to use the tin salts of the aforesaid acids in admixture with one another.

In preparing the drier, it is preferred first to wash the drier to completion, then to add the tin salt and subsequently to dehydrate the drier by heating, so as to prevent the risk that the tin salt is washed out and becomes inactive.

A small amount of tin salt suffices already to obtain a very light colored drier not liable to substantial darkening even when it is heated for a prolonged time to 120–150° C. It is preferred to use 0.05–2.0% by weight of tin metal in the form of the corresponding tin salt and calculated upon the solid drier. An amount outside the range indicated above, for example, 0.01% by weight or, for example, 3% by weight of tin salt may, however, also be used with good success. The salts of bivalent tin proved somewhat more effective than those of tetravalent tin, but the latter may also successfully be used.

A color-stabilizing drier of the type described above can be melted without undergoing darkening. This fact is of special importance for the removal of molten material from a drum.

Too dark, not color-stabilized driers which have been dissolved in organic solvents can be brightened to some extent by a subsequent addition of tin salts.

It can be observed during several weeks that the drier admixed with a tin salt is increasingly brightened. The brightening finally comes to a standstill and gradually decreases to some extent.

The color-stabilizing effect of the stabilizers used in this invention is indicated in Tables I to III below. The color indexes indicate in each particular case how many milligrams of iodine must be dissolved in 1 liter of an aqueous potassium iodide solution to bring about the same color impression as with the corresponding metal salt.

The color indexes indicated in Table I were obtained by dissolving solid, unstabilized, lead naphthenate in

TABLE I

Color-stabilization of lead naphthenate containing 15.5% by weight of lead with the tin salts of alpha-ethylhexanic acid or naphthenic acid, respectively

| Percent tin metal on lead naphthenate (solid): | Color index for stabilization with |                                     |
|------------------------------------------------|------------------------------------|-------------------------------------|
|                                                | tin salt of naphthenic acid        | tin salt of alpha-ethylhexanic acid |
| no addition (blank test)                       | not heated 20<br>Heated 250        | 20<br>250                           |
| 0.25% by weight tin                            | not heated 18<br>Heated 95         | 17<br>90                            |
| 0.5% by weight tin                             | not heated 18<br>Heated 52         | 16<br>25                            |
| 1.0% by weight tin                             | not heated 17<br>Heated 28         | 16<br>25                            |
| 2.0% by weight tin                             | not heated 16<br>Heated 25         | 16<br>22                            |

white spirit until the metal content was 15.5% by weight; the lead naphthenate was then color-stabilized.

The word "heated" as used in Table I is intended to mean that the specific specimen was kept for 3 hours at a temperature of 150° C. before the respective color index was determined.

It is obvious from the tables that the tin salts added prevented lead naphthenate from darkening upon heating. The untreated specimens establish that the tin salt exerts a subsequent brightening effect on lead naphthenate. For example, the addition of 2% by weight of tin metal, calculated on the solid lead naphthenate, reduces the color index from 20 to 16.

Table II indicates the color-stabilizing effect of various tin salts in the preparation of solid lead naphthenate (metal content: 31% by weight), of lead naphthenate dissolved in white spirit (metal content: 15.5% by weight), of solid zinc naphthenate (metal content: 12% by weight), and of zinc naphthenate dissolved in white spirit (metal content: 6% by weight).

TABLE II  
*Color-stabilization of lead naphthenate and zinc naphthenate with various tin salts*

| Product                                                              | metal content, percent by weight | stabilizer                                              | Percent Sn-metal on solid product | color index | color index after heating for 3 hours at 150° C. |
|----------------------------------------------------------------------|----------------------------------|---------------------------------------------------------|-----------------------------------|-------------|--------------------------------------------------|
| Lead naphthenate solid-----                                          | 31                               | unstabilized                                            |                                   | 140         | 180                                              |
|                                                                      |                                  | bivalent tin salt of alpha-ethylhexanic acid            | 0.3                               | 35          | 35                                               |
|                                                                      |                                  | bivalent tin salt of naphthenic acid                    | 0.3                               | 40          | 40                                               |
| Lead naphthenate dissolved in white spirit.                          | 15.5                             | bivalent tin salt of resinic acid                       | 0.3                               | 75          | 75                                               |
|                                                                      |                                  | unstabilized                                            |                                   | 15          | 110                                              |
|                                                                      |                                  | bivalent tin salt of alpha-ethylhexanic acid            | 0.3                               | 8           | 13                                               |
| Lead naphthenate solid-----                                          | 31                               | bivalent tin salt of naphthenic acid                    | 0.3                               | 9           | 16                                               |
|                                                                      |                                  | bivalent tin salt of resinic acid                       | 0.3                               | 27          | 60                                               |
|                                                                      |                                  | bivalent tin salt of alpha-ethylhexanic acid and        | 0.15                              | 40          | 40                                               |
| Lead naphthenate dissolved in white spirit.                          | 15.5                             | bivalent tin salt of naphthenic acid, mixed             | 0.15                              | 9           | 16                                               |
|                                                                      |                                  | bivalent tin salt of alpha-ethylhexanic acid and        | 0.15                              | 65          | 65                                               |
|                                                                      |                                  | bivalent tin salt of naphthenic acid, mixed             | 0.15                              | 10          | 43                                               |
| Lead naphthenate-----<br>Lead naphthenate dissolved in white spirit. | 15.5                             | tetravalent tin salt of naphthenic acid-----<br>do----- | 0.3                               | 150         | 190                                              |
|                                                                      |                                  | unstabilized                                            |                                   | 70          | 100                                              |
|                                                                      |                                  | bivalent tin salt of alpha-ethyl-hexanic acid           | 0.3                               | 65          | 110                                              |
| Zinc naphthenate solid-----                                          | 12                               | unstabilized                                            |                                   | 19          | 65                                               |
|                                                                      |                                  | bivalent tin salt of naphthenic acid                    | 0.3                               | 8           | 33                                               |
| Zinc naphthenate dissolved in white spirit.                          | 8                                | unstabilized                                            |                                   | 10          | 36                                               |
|                                                                      |                                  | bivalent tin salt of alpha-ethyl-hexanic acid           | 0.3                               |             |                                                  |
|                                                                      |                                  | bivalent tin salt of naphthenic acid                    | 0.3                               |             |                                                  |

The color indexes of Table I are far superior to those of Table II. This is due to the fact that in Table I the lead naphthenate used was prepared without a tin stabilizer; it was subsequently stabilized to demonstrate the color-stabilizing effect of the tin salt upon heating. In Table II the specimens had already been admixed with tin salts during their preparation.

In Table III two examples are compared one with the other in which the lead naphthenate solutions have been prepared by two slightly different processes. Details are given in the table.

TABLE III  
*Color-stabilizing effect of tin salts on lead naphthenate dissolved in white spirit (metal content 15.5% by weight) and prepared by two different processes*

| Preparation of the lead naphthenate solution                                                                                                                                    | stabilizer                                    | Percent Sn-metal on solid lead naphthenate | color index |
|---------------------------------------------------------------------------------------------------------------------------------------------------------------------------------|-----------------------------------------------|--------------------------------------------|-------------|
| Solid lead naphthenate prepared as usual by double reaction, dried.                                                                                                             | none                                          |                                            | 20          |
| Dissolved in white spirit and adjusted to metal content of 15.5% by weight.                                                                                                     | bivalent tin salt of alpha-ethyl-hexanic acid | 0.25                                       | 9           |
| Lead naphthenate prepared by double reaction in the presence of white spirit. Repeatedly washed with water and dehydrated by distilling off the water and part of white spirit. | none                                          |                                            | 18          |
| Adjusted to a metal content of 15.5% by weight with white spirit.                                                                                                               | bivalent tin salt of alpha-ethyl-hexanic acid | 0.25                                       | 8           |

Table III establishes that the tin salt exerts its stabilizing action notwithstanding the process used for making the lead naphthenate to be stabilized.

Obviously many modifications and variations of the present invention are possible in the light of the above teachings. It is, therefore, to be understood that within the scope of the appended claims the invention may be practiced otherwise than as specifically described.

We claim:

10. The process for stabilizing the light color of water-insoluble metal salts of organic acids which comprises preparing a homogeneous mixture of water-insoluble salts of metals selected from the group consisting of tin, lead, zirconium, cerium, lanthanum, zinc and calcium, said mixture containing as essential ingredients (1) a tin salt of an acid selected from the group consisting of naphthenic acids, resinous acids and  $\alpha$ -ethyl hexanic acid and (2) a member selected from the group consisting of salts, of one of the aforesaid metals other than tin, of naphthenic acids, of  $\alpha$ -ethyl hexanic acid, and mixtures

thereof, the tin salt being present in an amount by weight from about 0.01 to about 3.0%, calculated as metallic tin and referred to the amount of said other salts.

50. 2. A composition comprising a homogeneous mixture of water-insoluble salts of metals selected from the group consisting of tin, lead, zirconium, cerium, lanthanum, zinc and calcium, said mixture containing as essential ingredients (1) a tin salt of an acid selected from the group consisting of naphthenic acids, resinous acids and  $\alpha$ -ethyl hexanic acid and (2) a member selected from the group consisting of salts, of one of the aforesaid metals

other than tin, of naphthenic acids, of  $\alpha$ -ethyl hexanic acid, and mixtures thereof, the tin salt being present in an amount by weight from about 0.01 to about 3.0% calculated at metallic tin and referred to the amount of said other salts.

3. A composition comprising a homogeneous mixture of water-insoluble salts of metals selected from the group consisting of tin, lead, zirconium, cerium, lanthanum, zinc and calcium, said mixture containing as essential ingredients (1) a tin salt of an acid selected from the group consisting of naphthenic acids, resinous acids and  $\alpha$ -ethyl hexanic acid and (2) lead naphthenate, the tin salt being present in an amount by weight from about 0.01 to about 3.0% calculated as metallic tin and referred to the amount of said other salt.

4. The process as claimed in claim 1 wherein said

tin salt is present in an amount by weight from about 0.05 to about 2.0% calculated as metallic tin and referred to the amount of said other salts.

5. The process as claimed in claim 1, wherein the tin salt is added to said other metal salt after the latter has been washed.

6. A composition as claimed in claim 2 wherein said tin salt is present in an amount by weight from about 0.05 to about 2.0% calculated as metallic tin and referred to the amount of said other salts.

References Cited in the file of this patent

UNITED STATES PATENTS

15 2,236,296 Minich et al. ----- Mar. 25, 1941